

1

3,152,930  
PROCESS FOR PRODUCING MAGNETIC  
SHEET MATERIALS

Karl Foster, Wilkins Township, Allegheny County, Pa., assignor to Westinghouse Electric Corporation, East Pittsburgh, Pa., a corporation of Pennsylvania  
No Drawing. Filed Feb. 10, 1961, Ser. No. 83,276  
7 Claims. (Cl. 148—113)

This invention relates to an improved annealing process for obtaining double oriented or cube textured iron-silicon magnetic alloy sheets.

For a better understanding of the invention reference may be had to copending application Serial No. 85,432, filed January 27, 1961, now abandoned, and to the continuation-in-part thereof, application Serial No. 154,803, filed November 24, 1961, entitled, "Cube Textured Iron-Silicon Magnetic Alloy Sheets and Process for Making the Same," by G. W. Wierner et al., assigned to the assignee of the present application, wherein there is disclosed a novel iron-silicon alloy, particularly suitable for developing a double oriented magnetic structure. It is to the annealing treatment of alloys of the type described in the copending applications that the present invention is directed. The critical features set forth in the copending applications are that certain minimum amounts of sulfur must be present in the alloy sheets if the transformation to cube grain texture is to go to completion in the final annealing treatment.

As explained in detail in the copending application, the final annealing treatment is carried out in an atmosphere of very dry hydrogen or in vacuum. Under these conditions, the sulfur present in the alloy sheets which is necessary for successful transformation to cube texture, is rapidly lost with the result that the process of transformation may be prematurely arrested. The primary effort of this invention is directed to preventing such undesirable loss of sulfur from the sheets of iron-silicon alloy during the final annealing treatment.

In commercial practice the final annealing is carried out on sheet assemblies either in stacked form or in coils. The individual sheets, in the case of stacks of sheets, and the adjacent turns of the coil, in the case of coils, are separated from each other by a powdered medium, which is usually alumina,  $Al_2O_3$ , to prevent sticking. In accordance with the present invention the alumina powder is treated to provide sulfides which will contribute during final anneal a small but critical amount of sulfur adjacent the iron-silicon sheets to which it is applied.

It is an object of this invention to provide in the final annealing treatment of stacked or coiled iron-silicon alloy sheets a method for introducing sulfur into the area immediately adjacent the surfaces of the alloy sheet which comprises providing a thin layer of a sulfur-bearing  $Al_2O_3$  as the separating medium between sheets.

It is another object of this invention to provide a method for producing sulfur-bearing  $Al_2O_3$  which comprises exposing  $Al_2O_3$  powder to a hydrogen atmosphere containing a small amount of  $H_2S$  therein at an elevated temperature.

Still another object of the invention is to provide an  $Al_2O_3$  powder containing a small but critical amount of sulfur therein.

Other objects of this invention will, in part, be obvious and will, in part, appear hereinafter.

This invention is directed to a sulfur-bearing  $Al_2O_3$  powder which can supply sulfur to the surrounding environment at elevated temperature, to a method for preparing this sulfur-bearing  $Al_2O_3$  powder, and to a method for employing the sulfur-bearing  $Al_2O_3$  powder

2

in the final annealing treatment of iron-silicon base alloy sheets to promote transformation of a high volume of the sheets to cube grain texture.

More particularly, the sulfur-bearing  $Al_2O_3$  powder consists essentially of at least 0.001% sulfur, by weight, and the balance  $Al_2O_3$  except for small amounts of incidental impurities. Oxygen and readily decomposable oxides, such as water, carbonates and hydroxides should not be present in the alumina. A preferred range of sulfur content within the broad range stated above is from 0.005% to 0.02% by weight of sulfur.

The process for making sulfur-bearing  $Al_2O_3$  powder involves placing a quantity of the  $Al_2O_3$  in a furnace, heating the powder to a temperature in the range from 800° C. to 1300° C. for from 2 to 25 hours in a hydrogen atmosphere containing from 5 to 500 parts per million of  $H_2S$ . The temperatures of the heat treatment will drive off any water. The heat treated powder may then be stored in sealed containers until needed.

20 The method for the final anneal of stacked or coiled iron-silicon alloy sheet involves providing a thin separating layer of the sulfur-bearing  $Al_2O_3$  in an amount of at least from 1 to 10 grams per square foot of surface of sheet, between each sheet of the stack or between 25 adjacent turns of the coil, annealing the alloy sheet at a temperature from about 1100° C. to 1350° C. to affect substantially complete secondary recrystallization in an atmosphere capable of reducing or causing the disappearance of surface oxide films. The atmosphere 30 of the final anneal may be a very dry hydrogen having, for example, from —40 to —70° C. dew point or lower or a high vacuum of less than 10<sup>-2</sup> microns.

As a demonstration of the advantages of the use of the sulfur-bearing  $Al_2O_3$  powder of this invention, final 35 anneals were carried out on a heat identified as Number 8023, of which the following is a typical analysis of cold rolled sheets of final gauge:

| Percent Si<br>2.98 | Percent C<br>.003 | Percent N<br>.002 | Percent S<br>.001 | Percent O<br>.001 | Percent P<br>.001 | Percent Al<br>.003 |
|--------------------|-------------------|-------------------|-------------------|-------------------|-------------------|--------------------|
|--------------------|-------------------|-------------------|-------------------|-------------------|-------------------|--------------------|

The balance of the alloy was, of course, iron except for small amounts of incidental impurities. Material 45 of the above analysis had been arc melted cold rolled to .012 inch thick sheet and punched into laminations. The sheet material in this stage of the process had a rather poor surface finish which would normally be expected to impede cube grain growth. Therefore, some 50 of the laminations were polished with a mixture of 50%  $H_3PO_4$  (85%  $H_3PO_4$  concentration)—50%  $H_2O_2$  (30% concentration) to improve the surface condition. Two final annealing treatments for cube growth were used as described below following (A) a standard annealing treatment, and (B) an annealing treatment using the sulfur-bearing  $Al_2O_3$  of the present invention:

(A) 24 unpolished laminations and 12 polished laminations of the iron-silicon alloy were stacked between high temperature alloy plates of nickel-base alloy known as 60 Inconel with pure  $Al_2O_3$  powder interposed to separate the laminations and prevent sticking. The stack of laminations were heated in a tube furnace for 40 hours at 1200° C. in dry hydrogen having a dew point of —60° C.

(B) 45 polished and 45 unpolished laminations were 65 stacked between plates of nickel-base alloy, using sulfur-bearing  $Al_2O_3$  powder as a separating medium. The  $Al_2O_3$  powder had previously been heat treated for 16 hours at 1200° C. in a dry hydrogen atmosphere containing between 50 and 200 parts per million of  $H_2S$  gas. The stack of laminations was heat treated for 26 hours at 1200° C. in dry hydrogen having a dew point of —60° C.

In the tests, the alloy sheets to be treated by the process of the invention were clean and flat prior to heat treatment. Only an amount of  $\text{Al}_2\text{O}_3$  powder sufficient to prevent the sheets from sticking was used; a sieve was used to apply a thin uniform layer of powder of from 1 to 10 grams per square foot of surface area between the sheets. Amounts greater than 10 grams per square foot of surface are not necessarily detrimental. The stack was loaded uniformly so that there were no visible large spaces between the sheets. The loading was accomplished by tightening bolts which passed through the top and bottom nickel-base alloy plates. Each stack of laminations was packed in  $\text{Al}_2\text{O}_3$  powder and surrounded with nickel-base alloy (Inconel) plates to cut down the flow of gas against the laminations. The stack of laminations was heated at  $1200^\circ\text{C}$ . in the dry hydrogen for a time sufficient to provide complete secondary recrystallization and maximum attainable cube grain growth, usually between 4 and 24 hours.

In both tests the laminations underwent secondary recrystallization almost completely. The results of the above treatments were evaluated both on the basis of the volume percent of cube grains in the individual laminations as well as the percent of laminations of the total which were considered acceptable for use. The criterion used to decide whether a particular lamination was acceptable for use was that at least 80% of the volume of the lamination must be cube-on-face grains. The following results were obtained:

Table I

| Heat Treatment | Average volume Percent Transformed |          | Percent acceptable |          |
|----------------|------------------------------------|----------|--------------------|----------|
|                | Unpolished                         | Polished | Unpolished         | Polished |
| A-----         | 60                                 | 80       | 20                 | 70       |
| B-----         | 95                                 | 100      | 100                | 100      |

The results indicate the great improvement obtainable by using the sulfur-bearing  $\text{Al}_2\text{O}_3$  powder as a sheet separator in the final anneal. It is to be particularly noted that when the sulfur-bearing powder was employed, the cube texture secondary recrystallization grain growth in the iron-silicon alloy sheets is much less sensitive to surface conditions of the sheets.

In preparing the sulfur-bearing  $\text{Al}_2\text{O}_3$  powder a shallow layer of powder of from 80 to 150 mesh fineness, is placed in a nickel-base alloy boat in a furnace. The powder is heated to a temperature in the range from  $800^\circ\text{C}$ . to  $1300^\circ\text{C}$ ., and preferably about  $1200^\circ\text{C}$ ., for from 2 to 25 hours in a hydrogen atmosphere containing from 5 to 500 parts per million of hydrogen sulfide. Thus, in one successful process, hydrogen gas containing a concentration of  $\text{H}_2\text{S}$  of about 5 parts per million, flowing at about 10 cubic feet per hour, was passed over about 2 pounds of powder spread in a layer of  $\frac{1}{2}$  inch to  $\frac{3}{4}$  inch. At higher hydrogen sulfide concentrations shorter treating times and/or lower temperatures may be employed to effectively treat the  $\text{Al}_2\text{O}_3$  powder.

The sulfur-bearing  $\text{Al}_2\text{O}_3$  powder of this invention is analyzed by employing the following procedure: A 50 gram sample of  $\text{Al}_2\text{O}_3$  powder is placed in an ammoniacal zinc sulfate solution. The solution is then acidified by the addition of HCl to ensure the dissolution of all the sulfur in the powder. The solution is then titrated with a .01 N  $\text{KIO}_3$  solution. The total weight of sulfur in the  $\text{Al}_2\text{O}_3$  powder can then be calculated, and the sulfur is reported as a weight percentage of the  $\text{Al}_2\text{O}_3$  powder. A sample that had not been treated with  $\text{H}_2\text{S}$  showed no sulfur content by this test. A sample that had been treated for 16 hours in hydrogen containing 5 parts per million  $\text{H}_2\text{S}$  analyzed .009% by weight of sulfur. This sample was then used as the separating medium in a final anneal for transforming iron-silicon alloy sheets to cube texture at a temperature of  $1200^\circ\text{C}$ . in pure hydrogen

( $-70^\circ\text{C}$ . dew point) for 16 hours. When the  $\text{Al}_2\text{O}_3$  powder after the anneal was analyzed it contained 0.002% by weight of sulfur. Thus, it is demonstrable that during a final anneal of the type described sulfur is evolved from the  $\text{Al}_2\text{O}_3$ .

It is interesting to note that the sulfur content of the  $\text{Al}_2\text{O}_3$  powder deteriorates with time at room temperature in air. A sample showed the following characteristics with time.

| Days after treatment: | Percent S |
|-----------------------|-----------|
| 0 -----               | .012      |
| 1 -----               | .008      |
| 2 -----               | .002      |
| 5 -----               | .004      |
| 7 -----               | .001      |
| 8 -----               | .001      |

While some experimental fluctuations will be noted in the above data, it is clear that the sulfur content markedly declines over the test period.

It has also been observed that having the treated  $\text{Al}_2\text{O}_3$  open to relatively free circulation of air accelerates the decomposition noted in the previous table. The following results were obtained on another sample in which a part was kept in a sealed container and a part in a similar container with the cover open.

Table III

| Days on test | Percent S |
|--------------|-----------|
| 0 -----      | .007      |
| 4 -----      | .006      |
| 4 -----      | .003      |

The results given above indicate that that portion of the  $\text{Al}_2\text{O}_3$  powder which contains or is combined with sulfur decomposes with time in air.

It is believed that during the treatment of  $\text{H}_2\text{S}$  at  $1200^\circ\text{C}$ ., some of the  $\text{Al}_2\text{O}_3$  reacts to form  $\text{Al}_2\text{S}_3$  which is retained after cooling. During the final anneal treatment which has been described, the  $\text{Al}_2\text{S}_3$  reacts with hydrogen gas to form  $\text{H}_2\text{S}$  at the surface of the iron-silicon alloy sheets, which hydrogen sulfide at the sheet surface aids the cube growth process. It is known that  $\text{Al}_2\text{S}_3$  decomposes in moist air to form  $\text{H}_2\text{S}$ . Thus, it appears that air must be excluded from the treated  $\text{Al}_2\text{O}_3$  powder if it is to be stored for any length of time.

While applicant has advanced a proposed explanation for the phenomena observed he does not wish to be bound thereby, for other unknown factors may be at work in the process. The prime requirement is that sulfur is chemically associated with the  $\text{Al}_2\text{O}_3$  powder in such a way that it is available for the final annealing process. Where the term "sulfur-bearing  $\text{Al}_2\text{O}_3$ " is employed in this application, it will be understood to mean that the sulfur is chemically associated with the aluminum or alumina.

Table IV

EFFECT OF  $\text{H}_2\text{S}$  TREATED  $\text{Al}_2\text{O}_3$  ON CUBE GROWTH IN 3% Si-Fe

| Run No. | Treatment of $\text{Al}_2\text{O}_3$                           | Days after Treatment of $\text{Al}_2\text{O}_3$ before use in Annealing | Typical Wt., Percent S | Volume Percent Cube Grains |
|---------|----------------------------------------------------------------|-------------------------------------------------------------------------|------------------------|----------------------------|
| 70      | None                                                           | 0                                                                       | 0                      | 54                         |
|         | 16 hr. $1,200^\circ\text{C}$ . pure $\text{H}_2$               |                                                                         | 0                      | 55                         |
|         | 16 hr. $1,200^\circ\text{C}$ . $\text{H}_2+\text{H}_2\text{S}$ |                                                                         | .005 to .02            | 95                         |
|         | 16 hr. $1,200^\circ\text{C}$ . $\text{H}_2+\text{H}_2\text{S}$ |                                                                         | .001 to .002           | 80                         |
|         | After anneal (3)                                               |                                                                         | .001 to .002           | 77                         |
|         | After anneal (4)                                               |                                                                         | <.001                  | 61                         |
|         | 5 hr. $1,200^\circ\text{C}$ . $\text{H}_2+\text{H}_2\text{S}$  |                                                                         | .005 to .02            | 95                         |
|         | 3 hr. $1,200^\circ\text{C}$ . $\text{H}_2+\text{H}_2\text{S}$  |                                                                         | .003 to .007           | 85                         |
|         | 16 hr. $1,000^\circ\text{C}$ . $\text{H}_2+\text{H}_2\text{S}$ |                                                                         | .005 to .02+           | 99                         |

A series of final annealing treatments was made on a typical 3% silicon-iron alloy, identified as heat No. 1263. The typical analysis of this alloy is similar to heat No. 8023 set forth above with the difference that while 8023 had essentially no manganese, heat No. 1263 contains about 0.2% manganese. Table IV above shows data giving the amount of cube growth obtained in heat No. 1263 alloy sheets for different treatments of  $\text{Al}_2\text{O}_3$ .

The final annealing treatment used was 16 hours at 1200° C. in pure dry hydrogen (-70° C. dew point) and all annealing factors were kept constant. Run 1 was done with pure untreated  $\text{Al}_2\text{O}_3$  powder and shows that with a standard final annealing treatment only 54% cube grain growth took place in this alloy. Run 2 was made to show that high temperature purification of the  $\text{Al}_2\text{O}_3$  was not a factor, and it is clear that this had essentially no effect since the cube growth is approximately the same as in run 1. The above tests show that the  $\text{Al}_2\text{O}_3$  powder should contain between .005 and .02% sulfur, by weight, for the best results.

It is well known that final annealing treatments of the type with which this invention is concerned have also successfully been carried out in vacuum as well as in dry hydrogen. Sulfur is also required at the surface of the sheet during vacuum annealing to get good cube grain growth. If there is sufficient sulfur in the alloy sheet substantially complete cube transformation upon secondary recrystallization can be expected. But, because of the fugitive nature of sulfur under the conditions of a vacuum anneal, maintaining a desired sulfur concentration in the steel has been most difficult, with the result that cube texture transformation results have not been consistent. The use of sulfur-bearing  $\text{Al}_2\text{O}_3$  powder in vacuum annealing processes to obtain cube texture grain growth in iron-silicon alloy sheets has been as highly successful in vacuum annealing as it has been shown to be in hydrogen annealing.

The effect of sulfur-bearing  $\text{Al}_2\text{O}_3$  in vacuum annealing was demonstrated with a .008 inch thick sample of 3% silicon-iron, with essentially the same or similar alloy composition as those given above. In a standard vacuum anneal employing a vacuum of about .01 micron and using pure  $\text{Al}_2\text{O}_3$  for separating the sheets, only about 50% transformation to cube texture was obtained. For an identical anneal using sulfur-bearing  $\text{Al}_2\text{O}_3$  powder of the type described herein which contained about 0.007% sulfur, 100% transformation to cube texture was obtained in the same alloy sheet.

There has thus been described a relatively simple means for supplying sulfur to the atmosphere immediately adjacent the surface of iron-silicon alloy sheets undergoing final annealing treatment for transformation to cube texture. The sulfur-bearing  $\text{Al}_2\text{O}_3$  powder employed is easily made and readily employed in final annealing processes.

It is to be understood that all matter described herein is to be interpreted as illustrative and not as a limitation.

I claim as my invention:

1. In a final annealing treatment for iron-silicon alloy

sheet, the method for introducing sulfur into the area immediately adjacent the surface of the alloy sheet in an amount sufficient to promote cube texture grain growth comprising, providing a thin separator layer of sulfur-bearing  $\text{Al}_2\text{O}_3$  containing at least 0.001% by weight of sulfur on the surface of the alloy sheet, and annealing the alloy sheet in contact with said separator layer at a temperature of from 1100° C. to 1350° C. in an atmosphere capable of causing the removal of surface oxide films, for a period of time to cause substantially complete secondary recrystallization.

2. The method of claim 1 in which the atmosphere consists essentially of dry hydrogen having a dew point of at least -40° C.

3. The method of claim 1 in which the atmosphere is a vacuum of at least about 0.01 micron.

4. In a final annealing treatment for stacked or coiled iron-silicon alloy sheet, the method for introducing sulfur into the area immediately adjacent the surface of the

20 alloy sheet in an amount sufficient to promote cube texture grain growth comprising providing a thin separator layer of  $\text{Al}_2\text{O}_3$  powder containing from 0.005% to .02% sulfur, by weight, on the surface of the alloy sheet, and annealing the alloy sheet at a temperature of from 1100° 25 C. to 1350° C. in contact with said separator layer in an atmosphere capable of causing the removal of surface oxide films, for a period of time to cause substantially complete secondary recrystallization.

5. The method of claim 4 in which the atmosphere 30 consists essentially of dry hydrogen having a dew point of at least -40° C.

6. The method of claim 4 in which the atmosphere is a vacuum of at least about .01 micron.

7. In a method for treating an assembly or iron-silicon 35 alloy sheet material in coil or sheet form to obtain a high volume proportion of cube grains the steps comprising, finally annealing the assembly in a highly reducing atmosphere at a temperature of from 1100° C. to 1350° C. in contact with sulfur-bearing  $\text{Al}_2\text{O}_3$  containing at least 40 0.001% sulfur as the result of exposure to a hydrogen atmosphere containing from 5 to 500 parts per million of  $\text{H}_2\text{S}$  at an elevated temperature.

#### References Cited in the file of this patent

#### UNITED STATES PATENTS

|              |                 |               |
|--------------|-----------------|---------------|
| 1,226,750    | Chappell        | May 22, 1917  |
| 2,413,949    | Broverman       | Jan. 7, 1947  |
| 2,650,889    | Shannon         | Sept. 1, 1953 |
| 50 2,695,849 | McMullen        | Nov. 30, 1954 |
| 2,738,295    | McKnight et al. | Mar. 13, 1956 |
| 2,745,763    | Ueltz           | May 15, 1956  |
| 2,802,761    | Fast            | Aug. 13, 1957 |
| 55 2,948,644 | Ahrens          | Aug. 9, 1960  |
| 2,992,952    | Assmus et al.   | July 18, 1961 |

#### OTHER REFERENCES

Journal of Applied Physics, supplement to vol. 31, No. 5, May 1960 (pages 408S-409S relied upon).